

Oct. 21, 1930.

E. RICHTER ET AL

1,778,813

COATING SURFACES WITH CELLULOSE VARNISHES

Filed Sept. 11, 1928



Inventors:

Erich Richter

Walter Becker

By  
Bynes, Townsend & Bruckenstein  
Attorneys.

## UNITED STATES PATENT OFFICE

ERICH RICHTER, OF WOLFEN, KREIS BITTERFELD, AND WALTER BECKER, OF LEIPZIG, GERMANY, ASSIGNORS TO I. G. FARBENINDUSTRIE AKTIENGESELLSCHAFT, OF FRANKFORT-ON-THE-MAIN, GERMANY, A CORPORATION OF GERMANY

## COATING SURFACES WITH CELLULOSE VARNISHES

Application filed September 11, 1928, Serial No. 305,316, and in Germany August 24, 1927.

The present invention relates to improvements in coating surfaces with cellulose varnishes and for facilitating the application of more than one coating of cellulose varnish. 5 According to this invention surfaces, particularly of wood or metal, are prepared for the reception of cellulose varnishes by applying an intermediate coating consisting of a cellulose ester or esters of higher fatty acids, 10 if necessary with addition of colloid hydrocarbon exudations of plants, such as gums, gutta-percha, a resin, rubber, furthermore a colouring agent, a filling agent or the like.

Such an intermediate coating may also be 15 used when several coatings of cellulose varnish are applied. It is known that in the application of more than one coating of cellulose varnish, when a new layer is applied to that previously laid on, the solvent in the 20 varnish swells or partially dissolves the previous coating, even when the latter is completely dried. The attempt has been made to overcome this difficulty by selecting for the second coating a varnish the solvent of 25 which has the smallest possible solvent action on the varnish constituting the previous layer. This expedient, however, does not completely obviate the disadvantage. The attack of the 30 subsequently applied varnish on the previous layer can, however, be completely excluded by providing between the several layers of varnish of the usual kind, and particularly between the layer, applied by the pallet knife and the first layer an intermediate coating 35 consisting of a solution of a cellulose ester of a higher fatty acid or a mixture of such esters, if necessary containing a resin, rubber, a colouring matter, a filling agent or the like. Such intermediate layer or layers are applied 40 in the usual manner.

Examples of solutions suitable for producing intermediate layers according to this invention are as follows:

*Example 1.*—10 parts by weight of cellulose dilaurate and 8 parts of gutta-percha are dissolved in a mixture of 30 parts of benzene, 30 parts of xylene and 22 parts of chlorobenzene. The gutta-percha may be omitted if desired, or there may be substituted for it a 45 resin.

*Example 2.*—8 parts by weight of cellulose mono-acetate-distearate and 4 parts of rubber are dissolved in a mixture of 50 parts of di-chloromethane, 28 parts of chlorobenzene and 10 parts of benzene. The rubber 55 may be omitted if desired or a resin substituted for it.

Upon intermediate layers produced with such solutions any known cellulose varnish may be laid.

In the accompanying drawing cross sections of materials varnished according to our invention are shown on an enlarged scale. Figure 1 shows a base coated with an intermediate layer according to Examples 1 or 2, and with a cellulose varnish. In Figure 2 a base is shown coated with a plurality of cellulose varnish layers which may be different in their constitution, fastly combined together and with the base by intermediate layers containing a cellulose derivative of a higher fatty acid.

In the following claims the expression "surfaces" is intended to mean surfaces of wood or metal which may be unprepared or 75 coated with a layer applied by a brush or the pallet-knife.

What we claim is:

1. A process for preparing surfaces for the reception of cellulose varnishes by applying to the surface an intermediate coating of a solution containing such a cellulosic substance in which at least one OH group of the cellulose molecule is esterified by a higher fatty acid.

2. A process for preparing surfaces for the reception of cellulose varnishes by applying to the surface an intermediate coating of a solution containing such a cellulosic substance in which at least one OH group of the cellulose molecule is esterified by a higher fatty acid containing more than 10 carbon atoms.

3. A process for preparing surfaces for the reception of cellulose varnishes by applying to the surface an intermediate coating of a solution containing such a cellulosic substance in which at least one OH group of the cellulose molecule is esterified by lauric acid.

4. A process for preparing surfaces for the 100

reception of cellulose varnishes by applying to the surface an intermediate coating of a solution containing cellulose dilaurate.

5. A process for preparing surfaces for the reception of cellulose varnishes by applying to the surface an intermediate coating of a solution containing such a cellulosic substance in which at least one OH group of the cellulose molecule is esterified by a higher fatty acid and a colloid hydrocarbon exudation of plants.

6. A process for preparing surfaces for the reception of cellulose varnishes by applying to the surface an intermediate coating of a solution containing cellulose dilaurate and a colloid hydrocarbon exudation of plants.

7. A process for preparing surfaces for the reception of cellulose varnishes by applying to the surface an intermediate coating of a solution containing cellulose dilaurate and gutta-percha.

8. Materials lacquered with cellulose varnish coatings, said coatings covering intermediate layers which contain a cellulose derivative in which at least one OH group of the cellulose molecule is substituted by a higher fatty acid.

9. Materials lacquered with cellulose varnish coatings, said coatings covering intermediate layers which contain a cellulose derivative in which at least one OH group of the cellulose molecule is substituted by lauric acid.

10. Materials lacquered with cellulose varnish coatings, said coatings covering intermediate layers which contain a cellulose derivative in which at least one OH group of the cellulose molecule is substituted by a higher fatty acid, and colloid hydrocarbon exudations of plants.

11. Materials lacquered with cellulose varnish coatings, said coatings covering intermediate layers which contain cellulose dilaurate and gutta-percha.

45 In testimony whereof, we affix our signatures.

ERICH RICHTER.  
WALTER BECKER